

(Model.)

M. MANNESMANN.

2 Sheets—Sheet 1.

MANUFACTURE OF SEAMLESS TUBES.

No. 361,954.

Patented Apr. 26, 1887.

Fig. 1.



Fig. 2.



Fig. 3.



Fig. 4.



Fig. 5.



Fig. 6.



Witnesses:

Geo. H. Mabb

M. L. Adams

Inventor:

Max Manneumann,

Per Edw. E. Quincy,

Atty.

Model.)

M. MANNESMANN.

2 Sheets—Sheet 2.

MANUFACTURE OF SEAMLESS TUBES.

No. 361,954.

Patented Apr. 26, 1887.

Fig. 7.



Fig. 8.



Fig. 9.



Fig. 10.



Fig. 11.



Fig. 12.



Witnesses:

Geo. H. Heath

M. L. Adams

Inventor:

Max Mannesmann

Per Edw. E. Leinen

Atg.

# UNITED STATES PATENT OFFICE.

MAX MANNESMANN, OF REMSCHEID, GERMANY.

## MANUFACTURE OF SEAMLESS TUBES.

SPECIFICATION forming part of Letters Patent No. 361,954, dated April 26, 1887.

Application filed February 28, 1887. Serial No. 229,087. (Model.) Patented in Belgium August 14, 1886, No. 54,857, and in France August 19, 1886, No. 165,290.

To all whom it may concern:

Be it known that I, MAX MANNESMANN, of Remscheid, Germany, have invented certain Improvements in the Manufacture of Seamless 5 Tubing, of which the following is a specification.

This invention relates to a modification in the process of forming tubes from solid metallic ingots or blanks by the use of diagonally-acting-rolls, between the converging working-faces of which such ingots have been passed endwise.

The invention is based upon the discovery that by a suitable proportioning of the angles 15 of obliquity of the diagonally-acting rolls and the length and angles of convergence of their working-faces they will operate to develop a tubular formation in any part of a solid metallic ingot or blank which is submitted to 20 their action by causing a rupturing of the metal along the line of the geometric axis of such part and a radially-outward displacement of the metal therefrom, and hence that the whole of a solid ingot or blank of metal may 25 be transformed into a tube without the use of any mandrel for bearing against and holding back the central portion of the blank, or for assisting in the development of the tubular formation.

30 The proportioning and adjustment of the rolls are governed by the degree of softness and ductility of the metal which is to be operated upon; hence a different proportioning and adjustment of the rolls will be required for the 35 different metals, or even for the same metals at different heats.

It is to be observed that in the operation of diagonally rolling a metallic blank the blank is reduced in diameter by the convergence of 40 the working-faces of the rolls or rolling dies, in passing between which it is subjected to an endwise stretching, which is greater or less according as the direction in which the rolls act is more or less oblique. The blank is also 45 caused to rotate by reason of the opposite directions in which the dies act upon opposite sides of it.

Although not in all cases necessary, it is desirable, especially in the manufacture of iron 50 and steel tubes, that the portion of the blank on which the dies act shall have imparted to

it a progressively-increasing speed of rotation, so that the fibers of the metal will be made to extend spirally around the axis of the blank. Strong twist is given to the fibers for two purposes—to wit, to render the interior surface of the tube formed by the action of the rolls less rough and irregular, and to give the tube greater capacity to resist internal pressure. The desired twist is most effectually imparted 55 to the fibers by the employment of dies of such shape and arrangement that the diameters of the working-faces of the dies increase with greater or less rapidity from the place where they first engage the blank to the place where 60 they effect the greatest reduction in the diameter of the blank. To enhance the effectiveness of the dies in imparting this increasing twist to the metal operated upon, the working-faces of the dies are provided with projecting 65 ribs, or are otherwise so corrugated or roughened as to enable them to take a more effective hold upon the metal along the line of their impingement upon the blank, and thereby to move such metal in a spiral direction. 70

The desired rupturing effect and radial displacement of the metal from the center of the blank are most easily effected by the employment of two rolls or rolling dies, which act, respectively, upon diametrically opposite sides 75 of the blank. In passing between two dies the metal compressed in one direction by the squeezing action of the dies tends to expand in directions which are lateral to the line of compression, and as the blank revolves the 80 directions with relation to the blank of the planes of compression and expansion are constantly changing. Therefore in adjusting and proportioning the rolls the angles of convergence of their working-faces must be such as to 85 produce a suitably-moderate reduction in the diameter of the blank, and the obliquity of the direction in which the rolls act must be such that the stretching effect or the longitudinal movement imparted to the blank, while not 90 being too great nor too rapid to afford time for a sufficient number of rotations of the blank to bring about the central rupturing effect, will be commensurate with the tendency of the portion of the blank which is being operated upon to elongate itself while it is assuming the tubular form and the fibers are 95 100

acquiring their spiral positions in the shell of the tube. This can be more conveniently described in connection with the accompanying drawings and diagrams, which are as follows:

5 Figures 1, 2, 3, 4, 5, and 6 represent in central longitudinal section a solid metallic ingot or blank at different stages in its transformation into a tube during its endwise progress between two conical rolls, the axes of which are 10 oppositely inclined from the horizontal path through which the tube travels. Fig. 7 is a side elevation of the rolls, showing the blank in process of transformation into a tube. Fig. 8 is a diagram of the blank and rolls in trans- 15 verse section, indicating, theoretically, the effects of compression upon the metal and the direction in which the forces of compression are propagated from the places where the rolls impinge, respectively, upon the opposite sides 20 of the blank. Fig. 9 illustrates the effect of tensile stress in reducing the diameter of a uniformly ductile solid metallic bar. Fig. 10 illustrates the theoretical effect of tensile stress upon a metallic bar the center of which is 25 ruptured and the outer portion of which has been hardened by compression, and thus rendered less soft and ductile than the interior portion. Fig. 11 is a side view of a metallic bar or blank which has been circumferentially 30 grooved in the middle and chamfered at its ends; and Fig. 12 is a longitudinal section of the product resulting from the subjection of the form of blank shown in Fig. 11 to the action of the diagonal rolls, and in which, as will 35 be seen, the middle and end portions are solid and the portions intervening between the solid middle and ends are tubular.

For convenience of description it will be assumed that the two rolls shown in Fig. 1 and 40 the other corresponding figures are arranged, respectively, on either side of a horizontal path through which the blank travels; that the vertical planes of the axes of these rolls are parallel, and that their axes respectively are 45 oppositely inclined from the horizontal plane of the path through which the blank travels. It is also assumed that the conical portion of the side of each roll is at an angle of five degrees with its axis, and that the axial length 50 of the cylindrical portion of each roll is two and five-tenths inches and the axial length of the remainder or conical portion of each roll is five inches. It is assumed that the rolls are adjusted for operating upon a cast steel blank 55 which has been heated to a bright red heat, and that the original diameter of the blank is fifty millimeters, and that in passing endwise through the rolls its external diameter is diminished to thirty millimeters; hence that there 60 is a space of thirty millimeters between the cylindrical portions of the rolls where they most nearly approach each other.

In Fig. 1 the rolls are represented as having their working-faces provided with spiral corrugations. They may be otherwise corrugated or roughened in any way to prevent their slipping and to give them a more effective hold

upon the metal of the blank against which they impinge, whereby the displaced metal will be made to flow more nearly in the directions in which the rolls act. The corrugation or roughening of their surfaces improves the adaptability of the rolls to operate upon iron or steel blanks, and especially their capacity to impart the strong twist to the fibers of the metal which carries the fibers spirally around the shell of the tube formed by the action of the rolls, and thereby makes the interior surface of the tube smoother and the shell of the tube stronger.

In operating upon metals which are softer or more ductile than iron or steel, rolls having smooth working-faces may be employed.

The rolls A a rotate in the same direction, as indicated by the arrows A' a', and impart rotation in the opposite direction to the blank B, against the opposite sides of which the working-faces A<sup>2</sup> a<sup>2</sup> of the rolls respectively impinge.

For operating by means of rolls of the described dimensions the working-faces of which are arranged to have the described angles of convergence, the axes of the rolls require to have inclinations of from 1.8 to three degrees from the horizontal plane in opposite directions, accordingly as the metal operated upon is more or less hard. Such inclinations are indicated approximately in Fig. 1 and in the similar figures by the views which they each afford of the larger end, A<sup>3</sup>, of the roll A and of the smaller end, a<sup>3</sup>, of the roll a.

The drawings are not made to scale, but the described dimensions are given for the purpose of illustrating an example of proportion and adjustment of the rolls which is suitable 105 for effecting the transformation of a blank of cast steel fifty millimeters in diameter into a tube of thirty millimeters external diameter.

No attempt is made to represent the gearing by which the rolls are driven, nor any organized machine in which they are placed, nor any supports or guides for supporting and guiding the blank, because the machine forms no part of the present invention, and because diagonal rolling-machines provided with 110 guides for the object operated upon are already known.

The forces to which the blank is subjected in its passage between the diagonally-acting rolls are of complex character. The two rolls 120 act upon opposite sides of the blank with a kneading effect, compressing the metal against which they impinge to a certain depth beneath the surface. The cross area of the metal thus compressed is indicated approximately by the 125 section-lined triangles C C, shown in Fig. 8, which is a diagram of the blank in cross-section, representing the rolls arranged one above and the other beneath the blank.

The direction in which the forces of compression are propagated from the places where the rolls impinge upon the blank is indicated by the arrows which diverge from the section-lined triangles C C, respectively. It will be 130

seen that the resultant effect of these forces is to impart to the part of the blank under compression a tendency to expand laterally, as indicated by the horizontal arrows C' C' pointing outwardly from the center of the blank.

As the rolls are revolving in the direction indicated by the arrows A' a', and the blank of course revolving in the opposite direction, all parts of its circumference are in succession subjected to the kneading effect of the rolls, and thus the entire exterior of the blank is compressed and thereby hardened to a certain depth beneath the surface, and all parts of the interior of the blank are successively brought into the position in which they acquire the tendency to expand in the directions indicated by the arrows C' C'. The final effect of this tendency is to cause a rupturing of the blank along the line of its geometrical axis and the 15 radially-outward movement of the metal therefrom. There is, however, another influence exerted upon the blank which assists in imparting to it the tendency to become hollow. This is the longitudinal stretching effect to 20 which it is subjected by the rotation of the converging diagonally-acting rolls.

In Fig. 9 the familiar effect of tensile stress upon a solid metallic bar, E, is represented by the reduced diameter of the central portion, e. 30 In this case the metal is assumed to be uniformly soft and ductile throughout its entire mass and the fibers are assumed to have their ordinary adherence to each other.

Fig. 10 exhibits theoretically the effect of 35 tensile stress upon a bar of metal the fibers of which have been separated by a rupture extending along the line of the geometrical axis of the bar, and the exterior shell of which has been compressed and hardened to a certain 40 depth, while the interior portion retains the degree of softness which it originally possessed. In this case, as will be seen, the diminution in solid cross area of the central portion of the bar F resulting from the tensile stress exerted 45 upon it is due to the development of the cavity f in the interior of the bar. Fig. 10 may be regarded as an approximate representation of a bar the exterior portion of which has been compressed and hardened and the interior portion ruptured by the action upon it of the diagonal rolls.

The greatest hollowing effect is produced 50 when two rolls are employed, and when they act, respectively, on diametrically opposite sides of the blank, as illustrated in Fig. 8; but if, for any reason, it is desired to produce in the interior of the blank a hole of small diameter, the two rolls may be so arranged as not to act on diametrically-opposite sides of the blank, 55 or three rolls may be employed instead of two, in either of which cases the tendency of the blank to expand laterally induced by the compressive force of either one of the rolls will be to a greater or less extent counterbalanced by 60 the compressive force exerted by one or both of the other rolls.

In general, it is to be observed that the tendency of the solid blank to acquire the shape of a tube, and the inner diameter of the resulting tubular formation, depend, among other things, 70 upon the position of the blank between the two or three rolls which may be employed, and that the more nearly diametrically opposite the compressive forces exerted upon the blank the greater will be the tendency of the blank to 75 acquire a hollow form.

From what has been said it will be perceived that the angles of obliquity at which the diagonal rolls act and the angles of convergence and progressive variations in diameter of their 80 working-faces must be relatively so proportioned or adjusted as to impart to the portion of the blank which is being operated upon, during the time while it is being reduced from its original to its final diameter, a sufficient 85 number of revolutions to enable the rolls by their kneading action to effect the central rupturing of the blank, and by their progressive variability in diameter to impart the desired spiral twist to the reduced part of the blank, 90 and by their oblique action to exert the desired stretching effect, or, in other words, to impart the necessary longitudinal movement to the blank.

There are two ways of diminishing the number 95 of revolutions imparted to the blank while it is being reduced in diameter during its passage between the rolls. One is by making the convergence of the working-faces of the reducing-rolls more abrupt, and the other is by 100 increasing the angles of obliquity at which the rolls act without changing the angles of convergence of their working-faces; and, similarly, there are two ways of increasing the number of revolutions of the blank—either by 105 making the working-faces of the rolls less abruptly convergent or by changing the angles of obliquity at which the rolls act in such a way as to make them more nearly perpendicular to the axis of the blank; and it will of 110 course be seen that the two methods of changing the number of revolutions imparted to the blank—which consist of altering the angles of convergence of the working-faces of the rolls or of altering the angles of obliquity at which 115 the rolls act—may be employed either separately or together, as may be desired.

Variations in adjustment in the respects indicated will be required when there is a change 120 in the amount of reduction in external diameter to which the blank is to be subjected, and also when it is desired to effect a change in the interior diameter of the tubular formation. Thus, if it be desired to increase the internal diameter of the tubular formation, 125 the axes of the rolls will be so adjusted as to render the directions of their action more nearly perpendicular to the axis of the blanks, in which case while the reduction in the diameter of the blank is taking place the portion 130 of the blank acted upon will have imparted to it a greater number of revolutions,

which will make the pitch of the spirally-laid fibers finer and diminish the thickness of the shell of the tube.

What is claimed as the invention is—

1. The improvement in the art of transforming a solid metallic blank into a hollow body or tube, which consists in passing the blank endwise between the working-faces of diagonally-acting rolls so proportioned and adjusted as to progressively reduce the diameter of the blank to a prescribed extent while imparting to it a prescribed number of rotations, whereby the blank is progressively ruptured along the line of its axis and an outward movement of the metal from the center of the blank is concurrently induced.

2. The improvement in the art of transforming a solid metallic blank into a seamless tube and rendering the interior surface of such tube comparatively smooth, which consists in

progressively reducing the diameter of the blank, rupturing it along the line of its axis, and imparting to the portion of the blank acted upon a progressively-varying speed of rotation by means of suitably proportioned and adjusting diagonally-acting reducing rolls impinging upon different sides of the blank, substantially as herein set forth.

3. The product obtained by the method herein described as a new article of manufacture, the same consisting, essentially, of a rolled seamless tube constituted of a single integral bar of metal, the fibers of which are continuous and are overlaid spirally around the axis of the tube.

MAX MANNESMANN.

Witnesses:

ANNIE M. JONES,  
M. L. ADAMS.